

Dec. 19, 1922.

1,438,965.

A. McL. NICOLSON.

PIEZo-ELECTRIC DEVICE AND METHOD OF PRODUCING THE SAME.

FILED APR. 11, 1921.

2 SHEETS—SHEET 1.

Fig. 1.



Fig. 2.



Fig. 3.



Fig. 4.



Fig. 5.



Fig. 6.



Inventor:

Alexander M. Nicolson.

by J. G. Roberts Atty.

Dec. 19, 1922.

1,438,965.

A. McL. NICOLSON.

PIEZOELECTRIC DEVICE AND METHOD OF PRODUCING THE SAME,

FILED APR. 11, 1921.

2 SHEETS—SHEET 2.

Fig. 7.



Fig. 8.



Fig. 10.



Fig. 9.



Fig. 12.



Inventor:  
Alexander M. Nicolson.

by *J. G. Roberts* Atty.

## UNITED STATES PATENT OFFICE.

ALEXANDER MCLEAN NICOLSON, OF HILSDALE, NEW JERSEY, ASSIGNOR TO WESTERN ELECTRIC COMPANY, INCORPORATED, OF NEW YORK, N. Y., A CORPORATION OF NEW YORK.

## PIEZO-ELECTRIC DEVICE AND METHOD OF PRODUCING THE SAME.

Application filed April 11, 1921. Serial No. 460,396.

To all whom it may concern:

Be it known that I, ALEXANDER McL. NICOLSON, a subject of the King of Great Britain, residing at Hillsdale, in the county 5 of Bergen, State of New Jersey, have invented certain new and useful Improvements in Piezo-Electric Devices and Methods of Producing the Same, of which the following is a full, clear, concise, and exact description.

This invention relates to piezo-electric devices and methods of producing the same.

The invention aims to produce crystals having high piezo-electric activity and to 15 provide a sensitive, efficient, simple and durable piezo-electric crystal device for translating electrical variations into mechanical vibrations, and vice versa, and therefore capable of serving as a telephone transmitting or receiving device for instance.

Other objects of the invention will be apparent from the detailed description herein-after of the accompanying drawings.

Of the many mineral and organic crystals 25 investigated by H. and P. Curie and others, (see F. Pockels, Winkelmann's Handb. d. Phys., BD. IV, p. 783) the crystal of Rochelle salt (sodium potassium tartrate,  $\text{NaKC}_4\text{H}_4\text{O}_6\text{4H}_2\text{O}$ ) was found to have the 30 largest piezo-electric constant, approximately 10 electrostatic units per kg. Apparently no other crystal has yet been found to approach the piezo-electric activity of Rochelle salt, particularly if the crystal is 35 carefully chosen and specially prepared. It has been found that Rochelle salt is susceptible of greatly increased piezo-electric activity. An absolute electric charge of 200 electrostatic units per kg. pressure has been 40 obtained, resulting in potentials as high as 500 volts and alternating currents as high as 20 microamperes. Acoustic tones from a crystal may be heard at a distance of several hundred feet. Briefly the increased efficiency 45 is brought about by the following conditions:

1. Selection of particular habit of growth.
2. Desiccation.
3. Development of the crystal into a "composite" polar structure.

4. Application of static compression.
5. Use of electric poles normal to each other.

6. Application of torque.

These conditions will be considered in detail in connection with the drawings. 55

Fig. 1 of the drawings is a sectional elevation showing a vessel containing two crystals growing in accordance with a method comprised in this invention; Fig. 2 is a plan of 60 the apparatus and crystals shown in Fig. 1; Fig. 3 is a perspective view of a crystal grown in the manner indicated in Figs. 1 and 2; Fig. 4 is a sectional elevation showing a vessel containing a crystal growing in accordance with a second method comprised in 65 this invention; Fig. 5, is a plan of the apparatus and crystal shown in Fig. 4; Fig. 6 is a perspective view of a crystal grown in the manner indicated by Figs. 4 and 5; Fig. 7 is 70 a sectional elevation of a vessel containing a crystal growing in accordance with a third method comprised in this invention; Fig. 8 is a plan of the apparatus and crystal shown in Fig. 7; Fig. 9 is a perspective view of a 75 crystal grown in the manner indicated in Figs. 7 and 8; Fig. 10 is a perspective view of a piezo-electric crystal illustrating the hour glass marking appearing in crystals produced in accordance with the methods 80 comprised in this invention; Fig. 11 is an elevation, partly in section, of a piezo-electric crystal telephone receiving or transmitting device comprised in the invention; and Fig. 12 is a perspective view of the device 85 shown in Fig. 11, with the addition of a spirally corrugated cylindrical diaphragm.

Referring especially to Figures 3, 6, 9 and 10 which indicate the general appearance of crystals grown in accordance with this invention, the crystal surfaces may be classified into two systems of surfaces or zones which are normal to each other. One system of zones is parallel with the principal or crystallographic axis  $c$  and therefore encircles the crystal. The other system of zones comprises the two basal planes parallel with the  $a$  and  $b$  axes. In accordance with this invention the crystals are grown with the  $c$  and  $b$  axes in a horizontal posi- 100

tion as is indicated in Figures 1, 2, 4, 5, 7 and 8. This growth forms a particular habit, becoming dominant along the *c* and *b* axes, while development along the *a* axis upwards is partially suppressed on account of the super-saturation and consequent gradation in density of the liquor. This upward development may be completely suppressed by methods and for reasons pointed out hereinafter.

The crystals are grown from perfect nuclei possessing definite form and having *a*, *b* and *c* axes corresponding to the *a*, *b* and *c* axes respectively of the crystals shown in Figures 3, 6 and 9. In obtaining seed crystals, generally from a previous cropping, those seeds are selected in which growth along the *b* axis is fully developed (which happens when the seed nucleus grows with its *c* and *b* axes horizontal). These seeds are square, or nearly so, signifying that the growth along the *b* axis is about as great as, or greater than, that along the *c* axis. The thickness of the selected seed crystal along its *a* axis is generally  $\frac{1}{10}$  *b*. This dimension is a function of the density and head of the mother liquor.

In Figs. 1 and 2 the vessel 13 contains crystals 15 and mother liquor 17. The crystals rest on cylindrical, upwardly convex supports 19. The height of the supports and the depth of the mother liquor are so related that the surface of the mother liquor is at the level of the top of the crystal, whereby the upward growth of the crystal is prevented.

In growing a crystal, in the manner indicated in Figs. 1 and 2, a seedling 21 to the bottom of which a small quantity of wax or like adhesive has been applied is placed horizontally on top of the support 19 with the *c* axis of the seedling parallel to the surface of the support, the seedling and the mother liquor being between a temperature of 38° C. and 35° C., and the concentration of the mother liquor being such that the density of the solution at 50° C. would be about 1.33. The apparatus is then allowed to cool from between 38° and 35° C., to room temperature, for instance to about 20° C. On thus cooling rapidly the seed crystal will increase in size from a few grams weight to 50 or 500 grams according to the volume and density of liquor used. Growth occurs principally during the first 10 hours, although it may be continued several days during the condition of super-saturation if the crystal is allowed to remain in the mother liquor. An average size of crystal weighs 100 grams and its *b* and *c* axial lengths each approximate 65 mm., the proportions of the crystal being about those indicated in Figure 3. The cooling of the apparatus to room temperature ordinarily requires from about five to ten hours, the time being largely dependent on

the volume of mother liquor used. The rate of cooling is fairly rapid at first and tapers off as the temperature of the apparatus approaches the room temperature. The crystal usually grows to the desired size, for instance to such a size that it weighs about 100 grams, during this period of from five to ten hours, and may be taken from the mother liquor when it has attained such size. It appears probable that this rapid growth, due to the rapid cooling of the mother liquor causes the crystal to develop internal stresses producing strain regions symmetrical with the principal axis. The crystal thus acquires a composite structure closely related to the surface zones referred to above and to the electric poles to be developed in a manner which will now be set forth. At each end of the seed nucleus and along its *c* axis there appears a pyramid the base of which forms a polar terminal. The pyramids are not always very pronounced in the seed nucleus, but are more evident in the grown crystal after the latter has been desiccated as described hereinafter. The pyramids in the crystal are indicated at 23 in Figure 10. They consist of stratifications parallel to the *b* axis and normal to the *c* axis and to the remainder of the crystal structure, the stratification of which ordinarily is parallel with the *c* axis. The electrical performance of the crystal suggests that the crystal molecules throughout the pyramidal regions during growth are subject to forces which turn them, in planes containing the principal axis, through a right angle. This is indicated by the fact that the crystal, after subsequent treatment tending to render more pronounced these pyramidal terminations, develops its electrical poles (plus and minus corresponding with the conventional analogous and antilogous poles) in accordance with the two systems of zones referred to above. The poles are accordingly orthogonal, that is, at right angles to each other. This signifies that the bases of the pyramids, which occupy almost the entire area of the basal planes of the crystal, are electrically plus when the rest of the crystal structure is minus and vice versa. The effect becomes very pronounced when the crystal is subsequently desiccated in a manner which will now be described.

The desiccating treatment comprises submerging the crystal in 95% alcohol for about twenty-four hours, and 100% alcohol for about six hours, removing the crystal from the alcohol and subjecting it to low pressure and to heat. The alcohol should be brought to the temperature of the crystal before the crystal is introduced into it, in order that the crystal may not suffer stresses due to contact with a liquid of higher or lower temperature. The low pressure used for drying the crystal is preferably a pressure of about one

or two millimeters of mercury and the crystal is preferably subjected to the low pressure before it has been heated, and for a period of about 24 hours. The heating is 5 performed in an oven, at about 40° C. for a period of several days, or at a slightly higher temperature for a somewhat shorter period.

This treatment of the crystal is largely for removing waters of inclusion.

10 The crystal prepared in the manner described above will no longer be clear as when it was taken from the mother liquor, but will be cloudy or opalescent, the surface of the crystal showing irregular white spots 15 and the crystal exhibiting the pronounced "hour-glass" marking indicated at 23 in Fig. 10. The raw crystal as taken from the mother liquor possesses a large number of local electric poles which are variable in 20 their piezo-electric effect. The desiccated crystal is much stronger in effect and its electric poles are readily found in the case of the composite crystal to reside as described on the crystal surfaces with corresponding signs, respectively, in the zones parallel to the *c* axis and the zones normal to the *c* axis.

In order to prepare the crystal for piezo-electric use, a tinfoil electrode is pressed 30 around the girdle pole of the crystal and tinfoil electrodes are pressed on the basal planes, that is, the planes perpendicular to the *c* axis. The tinfoil is waxed on the side to be applied to the crystal, to make it 35 adhere closely to the crystal. Beeswax has been found suitable for this purpose.

Referring to Figure 11 (described in detail later) it will be noted that both basal planes 27 and 29 of the crystal 15 are slightly concave in the central or polar regions. 40 This feature is obtained in a crystal either by filing the basal planes of the crystal or by growing the crystal in a particular manner described hereinafter. The object of this feature is to render salient the ends of 45 the basal planes of the crystal. As pointed out in the article on the piezo-electric effect in the composite Rochelle salt crystal, by A. M. Nicolson in the proceedings of the 50 A. I. E. E., November, 1919, these ends of the basal planes are found to be mechanically sensitive regions of the crystal, just as were the ends of the basal planes of the corresponding crystal described in the U. S. patent application of Nicolson #295,967, filed May 9, 55 1919, entitled Piezo-electric transmitter. Rendering the diagonal corners of the crystal salient is for the purpose of insuring that when the crystal is mounted between 60 compressor plates such as 53 and 55 in the general manner indicated in Fig. 11, the pressure brought to bear on the crystal will be effective on these corners, so that stresses transmitted from the plates to the crystal 65 will be efficiently applied to the crystal.

Obviously, this purpose may also be realized by leaving the basal planes of the crystal flat and making the compressor plates concave toward the crystal.

For the purpose of obtaining an efficient 70 piezo-electric action at least two of these four diagonal corners at one crystallographic pole of the crystal should be perfect and flawless, apart from the composite structure referred to above.

75 As pointed out in the Nicolson article referred to above in the A. I. E. E. proceedings analysis of the direction of applied stresses to the sensitive regions described has shown that with crystals having the composite 80 structure referred to above a given force produces the greatest piezo-electric effect when the force is applied in such a way as to twist the crystal about its principal axis, and conversely, an applied electrical force produces the maximum mechanical response in the form of twisting motion, and therefore it is apparent that whether electrical or 85 mechanical results are to be produced from the crystal the torsional effect should be 90 utilized as far as possible, for instance as the graphophone transmitter described in the Nicolson application #295,967, referred to above utilized the torsional effect in a 95 piezo-electric crystal.

A crystal grown in the manner described above has a reentrant bottom face as shown 100 at 25 in Fig. 3, and due to the prevention of upward growth has but little thickness in the plane through the *a* and *c* axes. Due to this reentrant face and this thinness, the crystal is easily deformable by stresses torsional with respect to the principal axis of the crystal. It appears that the piezo-electric effect of the crystal is thereby greatly increased. The area of the basal planes or end 105 poles 27 and 29 should not be too small, and therefore, the crystal as a whole should not be too thin. Therefore, the cylindrical support 19 should not be too nearly flat.

110 An alternative method of growing the crystal is shown in Fig. 4, where a crystal 31 is shown growing in a vessel 33 which forms a mould for the crystal. The crystal and the vessel 33 are placed in the mother liquor in the vessel 35. The bottom of vessel 33 is convexed upward in order that the lower face of the crystal may be concave for the reason pointed out above. The depth of the mother liquor is so adjusted that upward 115 growth of the crystal is limited in order that the crystal may be readily deformable for the reason pointed out above. The vertical walls 37 of the vessel 33 normal to the principal axis of the crystal, are slightly concave inward except near their ends 39, in order that the basal planes 41 and 42 of the crystal may be slightly concave for the purpose pointed out above. The substantially vertical walls 38 of the mould or 120 125 130

vessel 33 flare slightly outwardly from bottom to top, to facilitate the removal of the crystal from the mould.

In Fig. 7, a crystal 51 is shown growing in a vessel 53 which forms a mould for the crystal since the vessel 53 is similar to the vessel 33. However, the vessel 53 is deeper than the vessel 33. The height of the mother liquor in the vessel 53 may be such that even after the crystal has grown to the desired size the top of the crystal is a considerable distance below the surface of the liquor, as shown in Fig. 7; or on the other hand the amount of mother liquor in the vessel 53 may be such that as the crystal grows and the level of the mother liquor therefore falls, the top of the crystal will reach the surface of the liquor so that further upward development of the crystal is prevented. Where the upward growth of the crystal is not prevented, the area of the basal planes is larger, as indicated in Figs. 7 and 9, but the crystal is not so readily deformable.

A piezo-electric crystal, such as 15 for instance, mounted as shown in Fig. 11 between two electrically conducting compressor plates such as 53 and 55 with its basal planes electrically connected together to form a pole of one sign, and its surfaces normal to the basal planes electrically connected to form a pole of opposite sign, may be used to translate mechanical vibrations into electrical vibrations or vice versa, the plates readily conveying jars and vibrations to the crystal. The members 53 and 55 are preferably of aluminum. With a crystal having a channel shaped face parallel to the principal axis a single tie-rod 59 lying within the channel formed by the concave face may be used to hold the crystal and the plates 53 and 55 in the desired relation. An insulating layer of rubber tape 66 may be wound upon this tie-rod. The rod may serve to electrically connect plates 53 and 55. The tie-rod is preferably riveted to one of the plates as shown at 60. The other plate may be slipped on the tie-rod and held against the crystal with the desired degree of pressure by means of a nut 62 threaded on the tie-rod. Or the latter plate may itself be threaded on the tie-rod, in which case the nut 62 is not essential but may serve to lock the plate in the position in which it exerts the desired degree of pressure on the crystal. A spring washer 64 is preferably interposed between the plate and the nut. The degree of static pressure exerted upon the crystal by the plates preferably corresponds to an absolute force of about 15 kg., since, as explained in the Nicolson application #295,967 referred to above and in the Nicolson article in the A. I. E. E. proceedings referred to above, the composite crystal is then most sensitive to variations of pressures applied so as to bear on the

salient ends of the basal planes simultaneously. This static pressure will ordinarily be sufficient to prevent slippage between the plates and the crystal when the crystal is being subjected to vibrations torsional with respect to its principal axis. However, a small quantity of dental cement or melted Rochelle salt or the like may be applied to the crystal and the plates along the lines of intersection of the plates with the crystal surfaces normal thereto, if necessary to prevent slippage between the plates and the crystal due to torsional stresses. If additional security be called for, short pins may be screwed into the plates to anchor the cement. The pins would preferably be placed one near each end of each of the basal planes of the crystal.

A binding screw 61 in one of the plates may be utilized for connecting one pole of the receiving or transmitting device to the circuits in which the device is to be used. To electrically connect the girdle electrode of the crystal with the circuits in which the transmitting or receiving device is to be used, several layers of tin foil are wrapped around the girdle electrode as shown at 63, and several turns of wire 65 are wrapped around the tin foil 63, several layers or wrappings of tin foil 67 and a layer of rubber tape 69 being then applied. The tie-rod 59 passes between the crystal and all of these wrappings. The wire 65 is preferably brought out from the device through an insulating bushing 71 in one of the plates 53 or 55.

As indicated above, the metal plates in Fig. 11 readily convey jars and vibrations to the crystal. The crystal and its mounting as shown in Fig. 11 therefore constitute an efficient generator or transmitter for converting the energy of sound waves into the energy of similar electrical waves. If this crystal transmitter be laid on a large sheet of paper and receivers be applied to the electrodes, sound produced by rubbing on the paper, or by the ticking of a watch, will be transmitted to the plates by the paper and can be heard in the receivers. Care should be taken that the tie-rod 60 does not protrude below plate 55, since when the transmitter plate 55 rests on a vibrating surface the vibrations are most efficiently transmitted to the crystal if the portions of the plate adjacent its perimeter are in intimate contact with the vibrating surface.

The device of Fig. 11 may also be used as a receiver, since the application of electro-motive force waves to its poles will produce corresponding mechanical vibrations of the two plates 53 and 55 in opposite rotational senses.

As indicated above, the crystal operates most efficiently as a translator of electrical into mechanical energy, or vice versa, when the vibrations to which it is subjected are, as far as possible, torsional with respect to the c

axis of the crystal. Thus, it has been found that the efficiency of the device shown in Fig. 11 may be materially increased by applying a cylindrical diaphragm 75 thereto as indicated in Fig. 12. This diaphragm should be of a strong light material such as gold beaters' skin or bond paper, and preferably consists of several layers of the bond paper. The paper is rolled around the periphery of disk 55 and clamped thereto by means of the clamp 77. The cylinder so formed by the paper is then twisted about its axis and clamped to the periphery of the disk 53 by means of the clamp 79. Spiral 15 corrugations 81 are thus formed in the paper diaphragm and when the device is used as a transmitter or electrical generator, mechanical stresses normal to the surface of the cylinder tending to vary the length of the cylinder produce torsional stresses in the crystal. When the device is used as a receiver, torsional vibrations electrically produced in the crystal twist the diaphragm, thereby efficiently setting up corresponding air vibrations.

As stated in the Nicolson article in the proceedings of the A. I. E. E. mentioned above, the crystal may be considered as a leaky condenser having a shunt resistance in excess of 100 megohms, and a capacity varying with the size of the crystal and usually of the order of  $10^{-9}$  F. The impedance of the crystal at acoustic frequencies varies from 100,000 to 300,000 ohms. If the crystal receiver is used with a microphone transmitter the supply potential for the crystal should preferably be stepped up to the crystal by means of a transformer. The motional impedance of the crystal may be found in the same manner as the motional impedance of an ordinary telephone receiver.

Properly articulated crystals may be grown much larger than is necessary for effective operation, but it is difficult to prevent cracks and flaws in drying and heating such large crystals. On the other hand, very small crystals are generally less effectively rendered "composite" on account of the relative absence of the stresses during shorter growing periods. Hence they are usually less efficient when mounted as described, and therefore it has been stated above that generally a crystal weighing about 100 gr. is a desirable size. However, it is at times desirable to use small crystals, for instance 5 or 6 mm. long and 2 mm. wide, as where the space available for the operating location of the crystal is very restricted.

Handling crystals grown in accordance with this invention sometimes causes the crystals to crack, especially if the crystals come into contact with the hands before the crystals have been desiccated as described above. This handling may be largely avoided by growing the crystals in a vessel such as

33 or 53 for instance, pouring off any excess mother liquor when the crystal has grown to the desired size, and allowing the crystal to remain in the vessel during desiccation. This method also has the advantage that shrinkage of the crystal during desiccation facilitates the removal of the crystal from the mould.

The expressions "cylindrical concave" and "cylindrical reentrant" and the like as used herein to describe crystal faces, are intended to apply to prismatic or other cylindrical hollowed out surfaces having a right section of a general arch or C shape, and the arch or C simulated may be as nearly a closed figure as desired. The expression "cylindrical convex" is used in a similarly broad sense. Where a crystal has a cylindrical upwardly convex lower face of which the right section is nearly a closed figure the crystal may be removed from its mould by sliding the crystal parallel to its c axis, the mould having no end walls. In some cases a reentrant face of a crystal may be such that its right section presents a plurality of sharply reentrant cusps superposed on the general line of reentrancy, for the purpose of making the crystal the more readily deformable by stresses torsional with respect to the c axis. Such a crystal face would, of course, be obtained by having a complementary face on the mould or support used in growing the crystal.

This application is a continuation of my applications Serial No. 226,343, filed April 2, 1918, Method of making piezo-electrical crystals; Serial No. 227,802, filed April 10, 1918, Piezophony; and Serial No. 295,967, filed May 9, 1919, Piezo-electrical transmitter, as regards common subject matter.

What is claimed is:

1. A piezo-electric crystal of sodium potassium tartrate, said crystal having a principal axis and having a cylindrical concave face parallel to said axis.
2. A piezo-electric crystal having a principal axis, said crystal having a channel shaped face parallel to said axis.
3. A piezo-electric crystal having a principal axis and having a reentrant cylindrical face parallel to said axis.
4. A piezo-electric crystal having a principal axis, every cross-section of said crystal normal to said axis having a reentrant side.
5. A piezo-electric crystal of sodium potassium tartrate having a principal axis, and having a face normal to said axis, one side of said face being reentrant.
6. The method of growing a piezo-electric crystal which comprises supporting said crystal in concentrated mother liquor, on the upwardly convex bottom of a vessel of such size that the grown crystal contacts

with two or more opposite vertical walls of said vessel.

7. The method of growing a piezo-electric crystal which comprises subjecting said crystal to the action of concentrated mother liquor in a vessel of such size that the grown crystal contacts with two or more opposite vertical walls of said vessel.

8. The method of growing a piezo-electric crystal which comprises subjecting said crystal to the action of concentrated mother liquor in a vessel of such size as to form a mould for the grown crystal.

9. The method of growing a piezo-electric crystal which comprises subjecting the crystal to the action of concentrated mother liquor and so adjusting the level of the surface of the mother liquor that said surface is at least as low as the top of the crystal while the crystal is growing.

10. The method of growing a piezo-electric crystal with opposed concave pole faces which comprises subjecting the crystal to the action of concentrated mother liquor in a vessel having opposed inwardly convex walls until the crystal moulds itself to the shape of said walls.

11. The method of growing a piezo-electric crystal which comprises supporting said crystal on a convex surface in a concentrated solution of mother liquor.

12. The method of growing a piezo-electric crystal which comprises supporting said crystal on a cylindrical convex surface in a concentrated solution of mother liquor.

13. The method of growing a piezo-electric crystal of sodium potassium tartrate which comprises subjecting the crystal to the action of mother liquor of a temperature of between 38° C. and 35° C. and of a density of about 1.33 at 50° C., and lowering the temperature of the mother liquor about 30° C. in less than ten hours.

14. The method of growing a piezo-electric crystal which comprises supporting the crystal on a cylindrical upwardly convex surface in mother liquor and increasing the concentration of the mother liquor at a rate such that the grown crystal possesses a pronounced composite structure.

15. The method of growing a piezo-electric crystal which comprises supporting said crystal on a cylindrical upwardly convex surface in concentrated mother liquor and lowering the temperature of said mother liquor about 30° C. in less than ten hours.

16. The method of growing a piezo-electric crystal of sodium potassium tartrate which comprises supporting said crystal on a cylindrical convex surface in mother liquor of a temperature of between 30° and 35° C. and of a density of about 1.33 at 50° C., and lowering the temperature of said mother liquor about 30° C. in from five to ten hours.

17. The method of preparing a piezo-electric crystal which comprises soaking said crystal in alcohol and subjecting said crystal to a pressure less than an atmosphere.

18. The method of preparing a piezo-electric crystal which comprises soaking said crystal in alcohol and subjecting said crystal to a pressure less than an atmosphere and to heat.

19. The method of preparing a piezo-electric crystal which comprises supporting a crystal of sodium potassium tartrate on a cylindrical convex surface in mother liquor of a temperature of between 38° C. and 35° C., and of a specific gravity of about 1.33 at 50° C., lowering the temperature of said mother liquor about 30° C. in from five to ten hours, removing said crystal from the mother liquor and soaking it in alcohol, removing said crystal from said alcohol and subjecting said crystal to a pressure less than an atmosphere and to heat.

20. The method of growing a piezo-electric crystal which comprises supporting said crystal, in concentrated mother liquor, on the upwardly convex bottom of a vessel of such size that the vertical walls of the grown crystal contact with the vertical walls of the vessel.

21. The method of growing a piezo-electric crystal which comprises subjecting a part only of said crystal to the action of supersaturated mother liquor.

22. The method of growing a piezo-electric crystal which comprises subjecting said crystal to the action of supersaturated mother liquor and maintaining a part of said crystal at least as high as the surface of said mother liquor while the crystal is growing.

23. A piezo-electric crystal having a principal axis and having a pronounced hour glass marking, said crystal having a channel shaped face parallel to said axis.

24. A piezo-electric crystal of sodium potassium tartrate, said crystal having a principal axis, said crystal comprising pyramids consisting of stratifications normal to said axis and to the remainder of the crystal structure, and said crystal having a channel shaped face parallel to said axis.

25. A piezo-electric crystal having an arch shape.

26. A piezo-electric crystal having a principal axis, said crystal having a shape such as to render the crystal readily deformable by stresses torsional with respect to said axis.

27. The method of growing a piezo-electric crystal of a predetermined shape which comprises subjecting said crystal to the action of concentrated mother liquor and limiting the growth of the crystal by a mould.

28. The method of preparing a crystal which comprises growing it in a mold and desiccating it before removal from the mold.

29. The method of preparing a piezo-electric crystal which comprises growing the

crystal in a mold and desiccating it in the mold by soaking it in alcohol and drying it internally.

30. The method of growing a piezo-electric crystal from a seedling which comprises supporting said seedling in a substantially horizontal position on a rigid extended surface in concentrated mother liquor at a tem-

perature of about 100° F. and allowing the mother liquor to cool to an ordinary room temperature in a period not greater than 10 hours.

In witness whereof, I hereunto subscribe my name this 8th day of April A. D., 1921.

ALEXANDER McLEAN NICOLSON.